

## UNITED STATES PATENT OFFICE

2,609,381

AMIDO-AMIDE DERIVATIVES OF DIBASIC  
ACIDS AND PROCESSES OF PREPARING  
THE SAME

Herman B. Goldstein, Cranston, and Stanley T. Clary, Coventry, R. I., assignors to Sun Chemical Corporation, Long Island City, N. Y., a corporation of Delaware

No Drawing. Application October 5, 1949,  
Serial No. 119,756

14 Claims. (Cl. 260—404.5)

1

The present invention relates to new organic compounds which are valuable as assistants in the treatment and finishing of textile materials.

One object of the present invention is to provide new water dispersible organic compounds useful for the treatment of textile materials which, upon such treatment, impart a highly improved hand and enhanced texture thereto.

Another object of the present invention is to provide new water dispersible organic compounds which are substantive to textile materials and which are highly resistant to ordinary laundering and dry cleaning methods after application thereto, thereby imparting a relatively permanent finish to such treated textiles.

Another object of the present invention is to provide new water dispersible textile finishing agents which do not cause discoloration nor yellowing of textile materials treated therewith, which are effective over long periods of time and under all the ordinary operations and conditions to which such textiles are subject, and which do not effect any color change in the shade of dyed fabrics, nor which deleteriously affect the light fastness of dyestuffs.

Other objects of the present invention will be apparent from the following description and appended claims.

It has been found that the above objects may be accomplished and that organic compounds having the properties and characteristics described therein may be prepared by reacting a high molecular weight aliphatic carboxylic acid, or derivatives thereof, such as the esters or halides thereof, with a polyamine to form an amido amine of such acid, and thereafter reacting the resultant amido amine with a dibasic acid, or a derivative thereof, such as the anhydride, esters or acyl halides thereof, in such manner that a disubstituted derivative of the dibasic acid is formed.

The organic compounds formed according to the process of the present invention may be considered to be disubstituted amido-amide derivatives of dibasic acids. Similarly, these products may also be considered to be acyl amides of a dibasic acid and high molecular weight aliphatic carboxylic acids.

The high molecular weight aliphatic carboxylic acids employed in preparing the above mentioned amido amines are those containing at least six carbon atoms in the aliphatic chain, as for example, caproic acid, caprylic acid and capric acid, and preferably those containing at least twelve carbon atoms in the molecule. Among those acids

which are preferred for use in the present invention are the higher saturated fatty acids such as lauric acid, myristic acid, palmytic acid, stearic acid, animal and vegetable oil saturated fatty acid compositions such as coconut fatty acids, and hydrogenated fatty acid compositions, such as from hydrogenated fish oils, hydrogenated cotton seed oil, hydrogenated soy bean oil and hydrogenated peanut oil. The higher unsaturated fatty acids as, for example, oleic acid, palmitoleic acid, linoleic acid, linolenic acid and eleostearic acid, may also be employed in preparing the compounds of the present invention. However, the use of such acids is not preferred since the end product, that is, the softener compound, displays a tendency toward slight discoloration due to the unsaturation in the finished product.

The polyamines which are reacted with the above mentioned acids to provide the amido amines which may be subsequently reacted with a dibasic acid to provide the new organic compounds of the invention, comprise those polyamines containing at least two amino groups of the primary or of the secondary type, and which may contain one or more aliphatic residues in the molecule. Examples of such polyamines include the diamines such as ethylene diamine, trimethylene diamine, tetramethylene diamine, pentamethylene diamine, and hexamethylene diamine; the polyethylene polyamines such as diethylenetriamine, triethylene tetramine, tetraethylene pentamine, etc.; substituted diamines such as ethyl ethylene diamine, hydroxyethyl ethylene diamine, N-N'dihydroxyethyl ethylene diamine, N-ethyl N'-aminoethyl ethylene diamine; and such other polyamines as diaminomethyl ether and diaminomethyl thioether.

Polyamines of the type exemplified above may be reacted with any of the previously mentioned aliphatic carboxylic acids to provide an amido amine containing at least one free primary or at least one free secondary amino group which is available for further reaction under proper conditions with the carboxyl groups of a dibasic acid, thus forming a diamide derivative of the said dibasic acid.

Among the various dibasic acids which, when treated with the amido amines under the conditions hereinafter set forth, will furnish the organic compounds of the present invention, may be listed, the aliphatic dicarboxylic acids such as oxalic acid, malonic acid, succinic acid, glutaric acid, adipic acid, pimelic acid, suberic acid and sebatic acid; the unsaturated aliphatic dicar-

2

boxylic acids such as maleic and fumaric acids; cyclic aliphatic dicarboxylic acids such as 1-4 cyclohexane dicarboxylic acid; and aromatic and alkyl aromatic dicarboxylic acids such as phthalic acid, isophthalic acid, homophthalic acid, and uvitic acid. Other dibasic acids, substituted or interrupted in their structure by hydroxyl, ester, ether and amino groups, or by halogen, oxygen and sulfur atoms may also be employed in the present invention. Some such acids are malic acid, tartronic acid, tartaric acid, 4 chlorophthalic acid, DL bromobutanedioic acid, aspartic acid, diglycolic acid, and dithioglycolic acid. The anhydrides, esters and acyl halides of the above mentioned dibasic acids may also be employed in carrying out the invention.

The compounds obtained in accordance with the procedures hereinafter outlined and with the materials above set forth may be represented by the following general formula:



In the above formula  $\text{R}_1$  and  $\text{R}_7$  represent an aliphatic chain containing five or more carbon atoms. Furthermore  $\text{R}_1$  and  $\text{R}_7$  may be identical or they may be different, depending upon whether the radicals represented by  $\text{R}_1$  and  $\text{R}_7$  are derived from the same acid or from different acids.

$\text{R}_2$ ,  $\text{R}_3$ ,  $\text{R}_5$  and  $\text{R}_6$  may represent hydrogen, a lower alkyl radical, or a lower hydroxyalkyl radical, the various substituents corresponding to the terminal substituents occurring in the particular polyamine employed.

$\text{R}_3$  and  $\text{R}_5$  may further represent an acyl residue of an aliphatic carboxylic acid. The particular compounds in which  $\text{R}_3$  and  $\text{R}_5$  have such representation occur, for example, in an amido amine in which the polyamine has been so reacted with an aliphatic carboxylic acid that both terminal amino groups contain an acyl radical and in which at least one of the acyl substituted amino groups contains a free hydrogen atom.

Depending upon the particular polyamine employed in preparing the amido amine,  $\text{G}$  in the above formula may be a secondary amino group, a simple lower alkyl or lower alkylol substituted amino group, oxygen or sulfur.

The letters  $a$ ,  $b$ ,  $c$ ,  $d$ ,  $e$  and  $f$  represent integers,  $a$  and  $c$  representing integers from 0 to 6; and  $b$ ,  $d$ ,  $e$  and  $f$  representing integers from 1 to 6.

That portion of the above general formula represented by  $\text{X}$  is a dicarboxylic acid residue in which  $\text{R}_4$  may represent an aliphatic group, a cyclo aliphatic group, an aromatic group or an alkyl aromatic group.  $\text{R}_4$  may also represent any of the said groups substituted within their structure by halogen, oxygen, and sulfur atoms, or by amino, ester, hydroxyl, and ether groups, or any of the said groups in which the carbon linkage is interrupted by halogen, oxygen or sulfur atoms, or by an amino, ester, hydroxyl, or ether group.

As has been set forth above,  $\text{X}$  in the general formula represents a dicarboxylic acid residue. The linkage between the two carbonyl groups contained in the said dicarboxylic group need not

necessarily be interrupted by any of the groups represented by  $\text{R}_4$  but may be a simple



linkage such as is had in oxalic acid. This type of linkage is obtained when oxalic acid is employed as the dibasic acid in the reactions set forth in the present invention. The resultant compounds therefore correspond to the general formula



wherein  $\text{X}$  represents the dicarboxylic residue of oxalic acid and wherein all the remaining substituents of the compound correspond to those of the preceding general formula as designated by the corresponding symbols therefor.

The compounds represented by the above general formula wherein  $\text{X}$  represents the dicarboxylic residue of oxalic acid, and methods of preparing the same are described in our copending patent application, Docket No. 328, filed on even date herewith.

The organic compounds of the present invention, as represented by the above illustrative formulas are prepared by reacting between approximately one mol to two mols of an aliphatic carboxylic acid containing at least six carbon atoms in the aliphatic chain with approximately one mol of a polyamine of the type previously described at a temperature between approximately 150°-180° C. until substantially complete reaction is obtained, and thereafter adding approximately one-half mol of a dibasic acid and further reacting the admixture at a temperature between approximately 150°-210° C., depending upon the particular reaction materials employed, until substantially complete reaction is secured as evidenced by the relatively low amine value of the reaction product. The products obtained in this manner, when cool, are generally tan colored, wax-like materials which are at least partially dispersible in hot water. In order to insure complete aqueous dispersion of the products of the present invention, it is generally preferable to add a solubilizing agent thereto, such as a lower alcohol, or a peptizing agent, such as an alkali, organic acid, a soap, etc.

Where the amido amine which is to be reacted with a dibasic acid contains more than one amino group in the molecular chain, more than one dicarboxylic acid residue may be introduced into the structure of the compound by increasing the molecular quantity of the dibasic acid in proportion to the molecular amount of the amido amine to be reacted. Thusly, where the symbol "a" and "c" in the above illustrative formulae are at least one and where  $\text{G}$  represents a secondary amino group, a second dicarboxylic acid residue may be incorporated into the structure of the compound, linking at least two of the amino groups represented by  $\text{G}$ . One example of such a compound and a method whereby the same is obtained are hereinafter set forth in illustrative Example 3.

The compounds of the present invention may

be worked up into a concentrated, water soluble softener paste, by treatment of the same with low molecular organic acids such as formic, acetic propionic, and lactic acids. Similarly, water soluble softener pastes which are particularly suitable for application to textile materials may also be prepared by treating the organic compounds obtained according to the processes of the present invention with caustic potash, caustic soda, and similar alkaline materials. Such pastes are usually prepared by heating the compounds to a temperature at which the said compounds are liquid and then adding the said low molecular acid or the alkaline material, as the case may be, plus an amount of water sufficient to obtain a paste of the desired consistency, and stirring the mixture until a smooth, homogeneous composition is obtained. Organic solvents, such as the alcohols previously mentioned, may also be added to the softener pastes to obtain improved solubility.

Illustrative of the preparation of the di-substituted amido amide derivatives of dibasic acids are the following illustrative examples. The quantities of all materials employed therein are set forth in parts by weight.

*Example 1*

276 parts of triple pressed stearic acid and 104 parts of hydroxyethyl ethylene diamine are heated together at 180° C. while removing the water which is formed by their interaction, until the acid value of the reaction mixture is reduced to approximately 5 mgm. KOH per gram. This reaction yields approximately 362 parts of a material which consists predominantly of a mixture of materials corresponding to the two formulas:



and



The above reaction mixture is kept at 180° C. while 67 parts of diglycolic acid are slowly added thereto. As the diglycolic acid is added, a reaction occurs with the evolution of water. After all the diglycolic acid has been added, the temperature of the reaction mixture is raised to approximately 190° C. and kept at that point until further reaction ceases. There is thus obtained approximately 400 parts of material which, at room temperature, is a dark tan, brittle, wax-like material having an acid value of approximately 30 mgms. KOH per gram and an amine value of approximately 25 mgms. KOH per gram. The reaction product thus obtained comprises predominantly a mixture of materials corresponding to the following formulas:



and



In preparing a softener paste suitable for the treatment of textiles, 35 parts of the reaction product obtained above are heated with 3 parts of 45% caustic potash and 62 parts of water, and the mixture stirred until uniform. There is obtained, when cool, a light tan colored, soft paste which is dispersible in hot water. When textiles are padded through a textile treating bath containing 1% of this paste, the fabric is made soft to the touch and has excellent draping qualities. This effect is substantially unaffected by washing or dry cleaning. When this product is applied to dyed fabrics it has no effect upon the color shade of the fabric, nor does it produce any deleterious effect on the light fastness of the dyestuffs in the fabric.

*Example 2*

To 362 parts of the reaction product of stearic acid and hydroxyethyl ethylene diamine, as obtained in Example 1, there are added 74 parts of phthalic anhydride while maintaining the temperature of the mixture at approximately 180° C. After all the phthalic anhydride has been added, the temperature of the reaction mixture is gradually raised to 190° C. and held at that point until the reaction ceases. There are obtained approximately 420 parts of a material which solidifies to a light tan colored wax-like material on cooling. The material thus obtained corresponds predominantly to the following formula:



The reaction product obtained above has a melting point of approximately 69° C.; the amine value, as determined by titration, is 40-50 mgms. KOH per gram.

Depending upon the equipment used and other factors influencing the reaction, it is sometimes necessary to add a small additional amount of phthalic anhydride to the reaction mixture to compensate for phthalic anhydride lost by sublimation, thus insuring substantial completion of the reaction. This is likewise true when using other dicarboxylic acids or derivatives thereof which tend to distill, sublime or decompose at the reaction temperatures used in the present processes.

The reaction product obtained above may be worked up into a water dispersible paste by stir-

7

ring 25 parts of the said reaction product with 4 parts of acetic acid and 71 parts of water, the temperature while mixing being sufficiently high to cause the reaction product to melt. When cool, the resultant paste is light tan colored and forms opalescent solutions when dispersed in hot water. Cotton fabrics or other textile materials upon immersion in a 1% aqueous solution of this paste, and subsequently dried, have a much softer hand than similar untreated fabrics. 5

### Example 3

276 parts of triple pressed stearic acid are mixed with 103 parts of diethylene triamine and the mixture slowly heated to 180° C. while passing nitrogen therethrough. When the evolution of water ceases, and the acid value of the reaction product has dropped to approximately 5 mgms. KOH per gram, there are then slowly added 110 parts of succinic acid while maintaining the temperature of the reaction mixture at approximately 185°-190° C. while continuing the passage of nitrogen through the mixture. After all the succinic acid has been added, the temperature is then further raised to 200°-210° C., and held in that range until the reaction is substantially complete. Upon cooling, a brown wax-like material is obtained which it is believed comprises in part a mixture of materials corresponding to the following formulas:



and



To prepare a softener paste, 20 parts of the product obtained as described above is heated with 75 parts of water and 5 parts of 47% caustic soda, and the mixture stirred until homogeneous. When further diluted with water to a concentration of approximately 1-10% and applied to textiles, this product imparts a soft feel to the cloth which is very fast to washing and dry cleaning.

### Example 4

225 parts of coconut fatty acids are heated with 148 parts of N,N' dihydroxyethyl ethylene diamine at 160° C. until the acid value of the reaction mixture drops to approximately 5 mgms. KOH per gram or less. The temperature of the reaction mixture is then raised to 180° C., and 74 parts of phthalic anhydride are slowly added thereto. When the addition of the phthalic anhydride to the reaction mixture has been completed, the temperature is further raised to 200° C. and held at that point until the reaction is completed. Upon cooling a tan colored wax-like

material is obtained, corresponding to the formula



wherein R represents the aliphatic residue of coconut fatty acids.

20 A textile softener paste may be prepared by stirring 20 parts of the reaction product of Example 4 in 80 parts of a 3% tallow soap solution. Textile materials, when treated with an aqueous textile treating bath containing a 0.5% solution of the softener paste, acquire a pleasingly soft feel. This effect is substantially unaffected by washing or dry cleaning.

### Example 5

284 parts of pure stearic acid is reacted with  
104 parts of hydroxyethyl ethylene diamine at  
170° C. until the acid value of the reaction product  
falls to less than 5 mgms. KOH per gram. The  
temperature of the reaction mixture is held at  
170° C. while 50 grams of anhydrous oxalic acid  
are added in small portions. Vigorous agitation  
is maintained during the addition of oxalic acid  
35 in order to break the foam which forms. When  
addition of oxalic acid has been completed, the  
temperature of the reaction mixture is raised to  
190° C. and kept at that point until the reaction  
is substantially completed, as indicated by an  
40 amine value less than approximately 30 mgms.  
KOH per gram. The reaction product thus ob-  
tained is a light tan colored wax-like material  
having a melting point of approximately 75° C.

55 and corresponds predominantly to the following formula:



65 A concentrated softener paste, using the reaction product of Example 5, may be prepared as follows.

70 35 parts of the said reaction product, 2 parts caustic potash, .02 part of an anti-foam agent, and 52.98 parts water are heated to 80° C. and stirred until a uniform composition is obtained. 10 parts of 99% isopropanol are then stirred in, and the mixture is allowed to cool. The resultant softener paste has a light tan color and forms opalescent solutions when dispersed in warm water. When a textile treating bath is prepared

9

with approximately 15 grams of the softener paste per liter of water, and textiles are treated therewith, a very soft, pleasing finish is imparted to the goods which is not noticeably affected by washing or dry cleaning. Moreover, the finish does not yellow or discolor white goods nor does it deleteriously affect the light fastness nor the color shade of dyed fabrics.

*Example 6*

To 370 parts of the pre-condensate prepared by the reaction of stearic acid and hydroxyethyl ethylene diamine as described in Example 5, there are slowly added 86 parts of diethyl fumarate while maintaining the temperature of the mixture at 150° C. When all of the diethyl fumarate has been added, the temperature of the mixture is slowly raised to 190° C., and is held at that point until substantially complete reaction has been obtained. When the reaction product has cooled, there is obtained approximately 410 parts of a dark brown, hard, wax-like material corresponding for the most part to the following formula:



A concentrated softener paste may be prepared by heating 25 parts of the reaction product obtained above with 5 parts of triethanolamine and 70 parts of water, and stirring the mixture until uniform. When this paste is further diluted with water to a concentration of approximately 1% to 10% and applied to textiles, particularly cellulosic textiles, a marked softening action on the fabric is obtained.

*Example 7*

290 parts of hydrogenated fish oil fatty acids are heated to 150° C. and approximately 90 parts of 70% ethylene diamine are gradually introduced below the surface of the molten fatty acids. After all the amine has been added the mixture is slowly heated to 170° C., and kept at that point until the acid value drops to approximately 10 mgms. KOH per gram. While maintaining the temperature of the reaction mixture at 170° C., 120 parts of sebacyl dichloride are slowly added thereto. There is a strong evolution of hydrogen chloride during this addition. After all the sebacyl dichloride has been added the temperature is raised to 200° C. while passing nitrogen through the mixture. Passage of the nitrogen through the mixture assists in removing the hydrogen chloride and helps to cause the reaction to go to completion more rapidly. The reaction product thus obtained corresponds to the following formula:



10

in which R<sub>1</sub> and R<sub>2</sub> represent the aliphatic residues of hydrogenated fish oil fatty acids.

When the amine value of the above reaction mixture drops to a minimum, the mixture is cooled to approximately 90° C. 15 parts of 45% caustic potash are then added thereto, followed by 1500 parts of hot water. The mixture is stirred until uniform, and is then allowed to cool. There is obtained approximately 1900 parts of a light tan colored paste. When this paste is further diluted with warm water and applied to textiles, a soft feel is imparted to the textiles. This softening effect is not materially affected by dry cleaning or washing.

*Example 8*

225 parts of coconut fatty acids and 116 parts of N,N'-diethyl ethylene diamine are heated together to a temperature of approximately 180° C., and the reaction mixture is maintained at that temperature until the acid value of the mixture drops to less than approximately 10 mgms. KOH per gram. To the resulting reaction product there are added, in small portions, 72 parts of phthalic anhydride. Upon completion of the addition of the phthalic anhydride to the reaction mixture, the temperature of the reaction mixture is gradually raised to approximately 200° C. and maintained at that point until reaction is substantially complete, as evidenced by a low amine value. Upon cooling to room temperature, a light, tan colored wax-like material is obtained.

In preparing a softener paste for the treatment of textiles employing the reaction product secured above, the molten reaction product is cooled to a temperature of approximately 100° C., and 40 parts of an aqueous 45% potassium hydroxide solution are added thereto. The mixture is stirred until homogeneous and there are then added thereto 1100 parts of hot water; stirring being continued until the mixture is again homogeneous. The resultant softener paste may then be dissolved in water in predetermined amounts to form a textile treating bath. When the softener paste is applied to fabrics such as, for example, spun rayon fabric, the fabric thus treated has a much softer hand than the untreated fabric, and this condition persists even after laundering and dry cleaning operations.

*Example 9*

288 parts of caprylic acid are heated to a temperature of approximately 140° C., and 74 parts of propylene diamine are gradually introduced thereto beneath the surface of the acid. The temperature of the mixture is then raised to approximately 180° C. and maintained thereat until reaction is substantially complete; as evidenced by an acid value of less than approximately 10 mgms. KOH per gram. Depending upon the equipment used and the conditions of the reaction, when using a relatively volatile amine such as propylene diamine, it is often found that a satisfactorily low acid value cannot be obtained by the use of the theoretical amount of the amine. In such case it is necessary to add an excess of the amine to compensate for the amine lost by vaporization. The reaction described above yields approximately 326 parts of a material which is substantially of the following formula:



11

The product thus obtained is dissolved in approximately 500 parts toluol and reacted therein with 91.5 parts hexanedioyl chloride at approximately 85° C. in the presence of a hydrogen chloride acceptor such as pyridine. At completion of the reaction, the reaction mixture is quickly transferred into boiling water and the mixture is agitated vigorously. Thereafter the water is drawn off and the toluol removed under vacuum conditions. There is thus obtained approximately 330 parts of a tan, semi-wax-like material, corresponding predominantly to the formula:



The product thus obtained may be dispersed in aqueous solution with caustic, alkali, or acetic acid in such manner as has been set out hereinbefore to form a softener paste which provides improved drape to textile materials when applied thereto and which has no adverse effect on the lightfastness properties of dyestuffs.

### Example 10

276 parts of triple pressed stearic acid are reacted with 104 parts of B,B'-diaminoethyl ether at 170° C. until the acid value of the reaction mixture drops to less than approximately 5 mgms. KOH per gram. The temperature of the reaction mixture is then raised to approximately 190° C.; then 59 parts of tartaric acid are added thereto in small portions. The temperature of the reaction mixture is maintained at this point until a substantially complete reaction has been obtained as indicated by the relatively low amine value of the reaction product. The reaction product consists predominantly of a compound having the formula



A concentrated textile softener paste may be prepared by heating 20 parts of the product of Example 10 with 75 parts of water and about 5 parts of 47% caustic soda, and stirring the mixture until homogeneous.

The hand and texture of textile materials treated with the compounds of the present invention are not only greatly improved over those of untreated fabrics, but the particular properties imparted to the fabric by the use of such compounds may be varied according to the specific compounds employed. For example, those compounds, in which the aliphatic chain portion represented by  $R_1$  and  $R_7$  in the illustrated general formulas is one containing less than 18 carbon atoms, impart exceptional softening effects to the fabric, while substantial bodying of the fabric with less softening effect is had when the compound employed in the treating bath is one

12

12  
in which the said aliphatic radicals consist of chains containing more than 18 carbon atoms. The particularly desirable properties imparted to the textile fabrics by the treatment thereof with the compounds of the present invention are substantially permanent due to the substantivity of these compounds toward textile materials, and particularly towards cellulosic fabrics. Due to the absence of primary amino groups in the compounds of the present invention, there is little danger of yellowing or discoloration of the fabric under conditions of heat, humidity, or long storage of the goods. As has been pointed out, the finishing agents of the present invention have no effect upon the color shades of dyed fabrics and do not adversely affect the light fastness of dyestuffs commonly used in coloring textile materials.

20 While the above products and processes of making the same constitute preferred embodiments of the present invention, changes may be made therein without departing from the scope of the invention as defined in the appended claims.

25 What is claimed is:

1. A chemical compound corresponding to the formula



where  $R_1$  and  $R_7$  are aliphatic chains containing at least 5 carbon atoms;  $R_2$  and  $R_6$  represent a radical of the group consisting of hydrogen, a lower alkyl radical, and a lower hydroxyalkyl radical;  $R_3$  and  $R_5$  represent a radical of the group consisting of hydrogen, a lower alkyl radical, a lower hydroxyalkyl radical, and an acyl group containing at least 6 carbon atoms;  $G$  represents a radical of the group consisting of an amino group, a lower alkyl substituted amino group, a lower alkylol substituted amino group, oxygen and sulfur;  $a$  and  $c$  represent integers from 0 to 6;  $b$ ,  $d$ ,  $e$  and  $f$  represent integers from 1 to 6;  $X$  represents a dicarboxylic acid residue in which  $R_4$  represents a member of the group consisting of aliphatic, cyclo aliphatic, aromatic, and alkyl aromatic groups; and any of the said groups containing in their structure a member of the class consisting of halogen, oxygen, and sulfur atoms, and amino, ester, hydroxyl and ether groups.

2. A chemical compound corresponding to the formula



70 where  $R_1$  and  $R_7$  are aliphatic chains containing at least 5 carbon atoms;  $R_2$  and  $R_6$  represent a radical of the group consisting of hydrogen, a lower alkyl radical, and a lower hydroxyalkyl radical;  $R_3$  and  $R_5$  represent a radical of the

13

group consisting of hydrogen, a lower alkyl radical, a lower hydroxyalkyl radical, and an acyl group containing at least 6 carbon atoms; *b* and *d* represent integers from 1 to 6; and where X represents a dicarboxylic acid residue in which R<sub>4</sub> represents a member of the group consisting of aliphatic, cyclo aliphatic, aromatic, and alkyl aromatic groups; and any of the said groups containing in their structure a member of the class consisting of halogen, oxygen, and sulfur atoms, 10 and amino, ester, hydroxyl and ether groups. 5

3. A chemical compound corresponding to the formula



where  $R_1$  and  $R_7$  are aliphatic chains containing at least 5 carbon atoms;  $R_2$  and  $R_6$  represent a radical of the group consisting of hydrogen, a lower alkyl radical, and a lower hydroxyalkyl radical;  $R_3$  and  $R_5$  represent a radical of the group consisting of hydrogen, a lower alkyl radical, a lower hydroxyalkyl radical, and an acyl group containing at least 6 carbon atoms;  $G$  represents a radical of the group consisting of an amino group, a lower alkyl substituted amino group, a lower alkylol substituted amino group, oxygen and sulfur; where  $a$  and  $c$  represent integers from 1 to 6; and where  $X$  represents a dicarboxylic acid residue in which  $R_4$  represents a member of the group consisting of aliphatic, cyclo aliphatic, aromatic, and alkyl aromatic group; and any of the said groups containing in their structure a member of the class consisting of halogen, oxygen, and sulfur atoms, and amino, ester, hydroxyl and ether groups.

4. Chemical compounds corresponding to the formula



where R is an aliphatic chain containing at least 5 carbon atoms.

5. Chemical compounds corresponding to the formula



where R is an aliphatic chain containing at least 5 carbon atoms.

14

## 6. Chemical compounds corresponding to the formula



15 where R is an aliphatic chain containing at least 5 carbon atoms.

7. Chemical compounds corresponding to the formula



30 where R is an aliphatic chain containing at least 5 carbon atoms.

## 8. Chemical compounds corresponding to the formula



where R is an aliphatic chain containing at least 5 carbon atoms.

45 9. A process for the preparation of a disubstituted amido amide derivative of a disbasic acid which comprises reacting the condensation product of an aliphatic carboxylic acid containing at least 6 carbon atoms and a polyamine, said condensation product containing at least one amino group which contains free hydrogen, at a temperature between approximately 150° C. to 210° C. with a member of the group consisting of aliphatic dicarboxylic acids containing at least 3 carbon atoms, aromatic dicarboxylic acids, alkyl aromatic dicarboxylic acids, cyclic aliphatic dicarboxylic acids, and anhydrides, esters, and acyl halides thereof.

60 10. A process for the preparation of a disubstituted amido amide derivative of a dibasic acid which comprises reacting an aliphatic carboxylic acid containing at least 6 carbon atoms with a polyamine at a temperature of 150° C. to 180° C.

65 to form a condensation product containing at least one amino group which contains free hydrogen, and thereafter reacting said condensation product at a temperature between approximately 150° C. to 210° C. with a member of the group 70 consisting of aliphatic dicarboxylic acids containing at least 3 carbon atoms, aromatic dicarboxylic acids, alkyl aromatic dicarboxylic acids, cyclic aliphatic dicarboxylic acids, and anhydrides, esters and acyl halides thereof.

75 11. A process for the preparation of a disub-

stituted amido amide derivative of a dibasic acid which comprises reacting the condensation product of an aliphatic carboxylic acid containing at least 6 carbon atoms and a polyamine, said condensation product having not more than one primary amino group, at a temperature between approximately 150° C. to 210° C. with a member of the group consisting of aliphatic dicarboxylic acids containing at least 3 carbon atoms, aromatic dicarboxylic acids, alkyl aromatic dicarboxylic acids, cyclic aliphatic dicarboxylic acids, and anhydrides, esters, and acyl halides thereof, to form a condensation product free of primary amino groups.

12. A process for the preparation of a disubstituted amido amide derivative of a dibasic acid which comprises reacting an aliphatic carboxylic acid containing at least 6 carbon atoms with a polyamine at a temperature of 150° C. to 180° C. to form a condensation product having not more than one primary amino group, and thereafter reacting said condensation product at a temperature between approximately 150° C. to 210° C. with a member of the group consisting of aliphatic dicarboxylic acids containing at least 3 carbon atoms, aromatic dicarboxylic acids, alkyl aromatic dicarboxylic acids, cyclic aliphatic dicarboxylic acids, and anhydrides, esters, and acyl halides thereof, to form a condensation product free of primary amino groups.

13. A process for the preparation of a disubstituted amido amide derivative of a dibasic acid which comprises reacting the condensation product of an aliphatic carboxylic acid containing at least 6 carbon atoms and a polyamine, said condensation product having no primary amino groups and not more than one secondary amino

group, at a temperature between approximately 150° C. to 210° C. with a member of the group consisting of aliphatic dicarboxylic acids containing at least 3 carbon atoms, aromatic dicarboxylic acids, alkyl aromatic dicarboxylic acids, cyclic aliphatic dicarboxylic acids, and anhydrides, esters, and acyl halides thereof, to form a condensation product free of primary and secondary groups.

14. A process for the preparation of a disubstituted amido amide derivative of a dibasic acid which comprises reacting an aliphatic carboxylic acid containing at least 6 carbon atoms with a polyamine at a temperature of 150° C. to 180° C. to form a condensation product having no primary amino groups and not more than one secondary amino group, and thereafter reacting said condensation product at a temperature between approximately 150° C. to 210° C. with a member of the group consisting of aliphatic dicarboxylic acids containing at least 3 carbon atoms, aromatic dicarboxylic acids, alkyl aromatic dicarboxylic acids, cyclic aliphatic dicarboxylic acids, and anhydrides, esters, and acyl halides thereof, to form a condensation product free of primary and secondary amino groups.

HERMAN B. GOLDSTEIN.  
STANLEY T. CLARY.

## 30 REFERENCES CITED

The following references are of record in the file of this patent:

## UNITED STATES PATENTS

35 Number Name Date  
2,425,393 Robinson et al. Aug. 12, 1947